

Patented Feb. 13, 1923.

## UNITED STATES PATENT OFFICE.

RICHARD WALTER, OF DUSSELDORF, GERMANY.

## METHOD FOR MAKING ACID-PROOF ALLOYS.

No Drawing.

Application filed July 16, 1920. Serial No. 396,863.

*To all whom it may concern:*

Be it known that I, RICHARD WALTER, a German citizen, and resident of Dusseldorf, Germany, have invented certain new and 5 useful Improvements in Methods for Making Acid-Proof Alloys, of which the following is a specification.

My invention relates to a method for obtaining acid-resisting alloys of silicon and 10 a heavy metal or metals, and particularly of silicon and iron.

As well known in the art the known iron-silicon alloys in their crystallized state are able to dissolve far less carbon than when 15 in liquid state, which phenomenon is still more pronounced with increasing silicon content. In consequence alloys of this character, on solidifying, separate out or disintegrate again that amount of carbon 20 which the liquid charge had incorporated beyond the eutectic, which segregation product is unfavorably known as "refining foam" and which seriously affects the homogeneity of the castings.

25. For this reason, and also for the purpose of reducing the undesirable hardness of the product, prior inventors kept the carbon content of these alloys as low as possible, only to find that the difficulties in economically manufacturing such alloys on a large 30 scale increase with the decreasing carbon content, and that it is practically impossible to produce substantially carbon-free alloys of this character.

35. By extended experiments I have now found that, contrary to prior knowledge, the hardness of the alloy decreases considerably as the carbon content rises, so that, for instance, with a silicon content of between 13 40 and 25%, and with a carbon content of not less than 0.65%, a decided softening occurs, and that if the carbon percentage is increased to 0.8% up to 1% a product results

which can readily be worked by chip-producing tools.

I have further found that these results are attained only if the crystallization is carried through in such manner that the formation of silicon cementite is prevented as much as possible and most of the carbon is changed 50 into its graphite modification. This is best attained by pouring the molten bath into the mold at a temperature just slightly above the fusing point of the alloy, whereas, if the bath is poured at a distinctly higher temperature, the formation of the hardening silicon cementite cannot be prevented.

The resulting alloy product is of very fine-grained homogeneous texture, and is relatively soft and easily workable.

What I claim is:—

1. The hereinbefore described method of making an acid-proof alloy containing heavy metal, a relatively high silicon content, and over 0.65% of carbon, which consists in 65 melting down said ingredients and pouring the molten bath at a temperature only slightly above the fusing point of the alloy.

2. The hereinbefore described method of making an acid-proof alloy, composed of 70 iron, a relatively high silicon content, and over 0.65% of carbon, which consists in melting down said components and pouring the bath at a temperature only slightly above the fusing point of the alloy.

3. The hereinbefore described method of making an acid-proof alloy, which consists in melting together heavy metal, silicon and carbon, the silicon content being within the limits of 13% and 25%, and the carbon content in excess of 0.65% of the total, and casting the molten bath at a temperature slightly above the fusing point of the alloy.

In testimony whereof I affix my signature.

RICHARD WALTER.